

## UNITED STATES PATENT OFFICE

2,208,218

## LUBRICATING OIL PREPARATION

Herman P. Lankelma, Cleveland, Ohio, assignor to  
 The Standard Oil Company, Cleveland, Ohio, a  
 corporation of Ohio

No Drawing. Original application September 4,  
 1936, Serial No. 99,450. Divided and this ap-  
 plication June 7, 1938, Serial No. 212,292

8 Claims. (Cl. 252—51)

This invention relates to lubricating oils, and  
 more particularly the beneficiation of mineral  
 lubricating oils which are subject to high tem-  
 perature usage; and it is among the objects of  
 5 the invention to provide an oil which is especially  
 durable in high temperature usage, as in internal  
 combustion engines, etc.

To the accomplishment of the foregoing and  
 related ends, the invention, then comprises the  
 10 features hereinafter fully described, and par-  
 ticularly pointed out in the claims, the following  
 description setting forth in detail certain illus-  
 trative embodiments of the invention, these be-  
 15 ing indicative however, of but a few of the va-  
 rious ways in which the principle of the invention  
 may be employed.

A mineral lubricating oil stock of desired vis-  
 cosity is treated by incorporation of a small  
 20 amount of a hydro-compound from the group  
 consisting of hydroquinine, hydroquinidine and  
 hydrocinchonine. These compounds readily dis-  
 solve and disseminate, and the amounts em-  
 ployed may in general be from 0.001 to 5 per  
 25 cent, and oil stocks of for instance 45-200 sec.  
 at 210° F. Saybolt Universal may be treated.

As an example: 0.01 per cent of hydroquinine  
 is incorporated in an oil of 50 sec. at 210° F. Say-  
 bolt Universal, being thoroughly mixed.

Similarly with the other hydro-compounds.  
 30 This application is a division of my applica-  
 tion Ser. No. 99,450, filed Sept. 4, 1936.

Other modes of applying the principle of the  
 invention may be employed, change being made  
 35 as regards the details described, provided the fea-  
 tures stated in any of the following claims, or  
 the equivalent of such, be employed.

I therefore particularly point out and dis-  
 tinctly claim as my invention:

1. A process of preparing lubricating oils,  
 40 which comprises beneficiating a mineral oil ca-

pable of lubricating viscosity at high tempera-  
 ture by incorporating therewith a small amount  
 of a hydro-compound of the group consisting of  
 hydroquinine, hydroquinidine, and hydrocin-  
 chonine. 5

2. A process of preparing lubricating oils,  
 which comprises beneficiating a mineral oil ca-  
 pable of lubricating viscosity at high tempera-  
 ture by incorporating therewith a small amount  
 of hydroquinine. 10

3. A process of preparing lubricating oils,  
 which comprises beneficiating a mineral oil ca-  
 pable of lubricating viscosity at high tempera-  
 ture by incorporating therewith a small amount  
 of hydroquinidine. 15

4. A process of preparing lubricating oils, which  
 comprises beneficiating a mineral oil capable of  
 lubricating viscosity at high temperature by in-  
 corporating therewith a small amount of hydro-  
 cincinonine. 20

5. A lubricating composition comprising a  
 mineral oil capable of lubricating viscosity at  
 high temperature and a small amount of a  
 hydro-compound of the group consisting of  
 hydroquinine, hydroquinidine, and hydrocin-  
 chonine. 25

6. A lubricating composition comprising a  
 mineral oil capable of lubricating viscosity at  
 high temperature and a small amount of hydro-  
 quinine. 30

7. A lubricating composition comprising a  
 mineral oil capable of lubricating viscosity at  
 high temperature and a small amount of hydro-  
 quinidine. 35

8. A lubricating composition comprising a  
 mineral oil capable of lubricating viscosity at  
 high temperature and a small amount of hydro-  
 cincinonine. 40

HERMAN P. LANKELMA.